

May 16, 1961

M. N. ORNITZ ET AL

2,984,473

FURNACE CONVEYOR ROLLS AND THE LIKE

Filed July 14, 1958

Fig. 1.



Fig. 4.

Fig. 2.



Fig. 3.



INVENTORS

Martin N. Ornitz &  
Ray H. English

*By Hayes, Leonard & Buell  
Their Attorneys*

# United States Patent Office

2,984,473

Patented May 16, 1961

1

2,984,473

## FURNACE CONVEYOR ROLLS AND THE LIKE

Martin N. Ornitz, Wilkinsburg, and Ray H. English, McCandless Township, Allegheny County, Pa., assignors to Blaw-Knox Company, Pittsburgh, Pa., a corporation of Delaware

Filed July 14, 1958, Ser. No. 748,320

8 Claims. (Cl. 263—6)

This invention relates to furnace conveyor rolls and the like and particularly to furnace conveyor rolls over which metallic strip is passed and advanced through a heating furnace.

The invention will be particularly illustrated and described as embodied in a furnace conveyor roll for passing steel strip through an annealing furnace. It is well known in the metal treating arts that difficulties are encountered by reasons of the collection of accretions of material from metal strip on the metallic conveyor in the heating furnace, e.g., metallic conveyor elements used in annealing strip with the strip passing over or around the rolls. The problem has been, particularly, acute in the treatment of high silicon steels and other steels which require high treatment or annealing temperatures. This problem appears to be influenced by a variety of factors including the tension of the strip, the composition of the strip, the temperature of the furnace atmosphere, as well as the characteristic of the roll surface. Various attempts to solve this problem have been heretofore proposed, such as, coating the surface with various materials resistant to the formation of accretions, however, these coatings heretofore proposed have been subject to the difficulty of spalling when the temperature changed materially in the furnace and, particularly, where the furnace was cooled down between runs. This spalling problem has, in some instances, been almost as bad as the original problem of the formation of the accretions.

We have invented a conveyor roll and the like which overcomes both the problems of accretions forming on the surface, as well as the problem of spalling. The conveyor roll of the present invention has a structural metal body with a stabilized zirconia work engaging surface. Preferably, the body of the roll is of metal; a high temperature alloy of known composition desirably being employed. We have found that the zirconia used for the work engaging surface must be stabilized with calcium oxide or an equivalent stabilizing agent. Unstabilized zirconia has proven unsatisfactory and is subject to the spalling problem, previously mentioned. Preferably, the metal roll is provided with a coating or film of Nichrome prior to the addition of the stabilized zirconia coating. We have found that the interposition of the Nichrome film on the roll improves the life of the stabilized zirconia surface over that of zirconia alone on ferrous base rolls. The metal roll body may be a hollow body such as that commonly used in conveyor rolls or it may be of any other roll design.

In the foregoing general description we have attempted to set out certain of the problems of the furnace conveyor roll art together with certain objects, purposes, and advantages of our invention. Other details, purposes, objects and advantages will be apparent from the following description of a present preferred embodiment of the invention and the accompanying drawings in which:

Figure 1 is a diagrammatic view of a heat treating chamber showing that a high strip can be supported on the furnace conveyor rolls of this invention;

2

Figure 2 is a view partly in elevation and partly coaxial with the roll;

Figure 3 is a perspective view of the furnace conveyor roll of Figure 2 shown as having its work engaging surface sprayed with stabilized zirconia; and

Figure 4 is a diagrammatic fragmentary cross section to enlarged scale of a part of the roll body of Figure 2.

Referring to the drawings, we have illustrated a furnace chamber 10 through which strip 11 is adapted to be drawn,

- 10 the strip passing over a series of rolls 12 at the top of the furnace and then passing over rolls 12 at the bottom of the furnace. It is desirable that the rolls be of uniform construction. The rolls 12 may be driven or turned idly as the strip passes through the chamber 10. The chamber 15 10 is heated internally by suitable heating methods not illustrated herein.

Referring more particularly to Figures 2 and 3, the furnace conveyor roll 12 includes a metal body 13 made up of a barrel 14, two shaft ends 15, and two closure plates

- 20 16. The shaft ends 15 are filled with heat insulating material 17. The barrel 14 and shaft ends 15, and the closure plates 16 may be of any suitable alloy such as is used in the manufacture of furnace conveyor elements. Preferably we use a heat resistant alloy. The barrel 25 14 has a thin film of Nichrome 18 applied to its outer surface. This film may be applied by any conventional means, as for example, spraying. The outer work engaging surface coating 20 of stabilized zirconia is then applied to the Nichrome. Here again the coating may be applied by any known method which will provide a fused surface. For example, the stabilized zirconia may be applied by high temperature spraying and to this end a metallizing gun 19 is provided to melt and spray the stabilized zirconia.

- 30 35 The shaft ends 15 have cylindrical portions 21 fitting within the ends of barrel 14, tapered portions 22, cylindrical end portions 23 and trunnions 24 which may be mounted for rotation in a conventional manner.

- The ends of the barrel 14 are welded to the ends of the 40 shaft ends 15 by weldments 25. The closure plates 17 are welded to the shaft ends 15 by weldments 26.

- The stabilized zirconia surface 20 constitutes the working engaging surface of the roll and is the only portion of the roll which comes in contact with the strip being carried over the roll.

The advantages of the present roll are perhaps best illustrated by the following test.

- A ferrous roll body containing 25% chromium and 12% nickel was spray coated over  $\frac{1}{2}$  of its length with 50 a film of 80-20 Nichrome (80% nickel and 20% chromium). A coating of stabilized zirconia (zirconia stabilized for example with CaO) was applied to  $\frac{1}{3}$  of the Nichrome coated length. A coating of alumina was applied to another third of the Nichrome coated length

- 55 and a coating of zirconium silicate was applied to the remaining  $\frac{1}{3}$  of the Nichrome coated length. Identical coatings of stabilized zirconia alumina and zirconium silicate were applied to the portions of the roll which did not have the Nichrome coating. The roll was then subjected to cycles of temperature change such as would be encountered in heating and cooling a strip treating furnace.

- 60 After the first cycle the alumina had spalled on both Nichrome coated and uncoated areas to an extent that it would be unsatisfactory for further use. The zirconium silicate showed signs of spalling in both cases but could still be used. After the second cycle only the stabilized zirconia on the Nichrome film remained intact. After five cycles all of the coatings had spalled off except the stabilized zirconia which still remained unimpaired.

Another roll of nickel base alloy containing 48½% Ni, 28% Cr, 15½% Fe and 5% W was coated directly

with stabilized zirconia on  $\frac{1}{2}$  of its length and with alumina over the other  $\frac{1}{2}$  of its length. The roll was then subject to heating and cooling cycles. Again, the alumina spalled off to an extent that it would be unsatisfactory for further use after the first cycle whereas the stabilized zirconia remained unimpaired after five cycles.

It is apparent from the foregoing examples that stabilized zirconia work surfaces on conveyor rolls will overcome the difficulties of spalling heretofore experienced. The stabilized zirconia coating must be applied to a roll body of proper composition and physical properties for the temperature in the particular furnace involved. The zirconia coat may be used in certain cases without an undercoat, however, where any difficulty with spalling is encountered a Nichrome film applied to the roll surface prior to the application of the stabilized zirconia will eliminate the spalling problem.

While we have illustrated and described a present preferred embodiment of our invention it will be understood that the invention may be otherwise embodied within the scope of the following claims.

We claim:

1. A furnace conveyor roll and the like comprising a work supporting metal body and a coating of stabilized zirconia covering the work engaging portion of said body and being fixed thereto.
2. A furnace conveyor element and the like comprising a work supporting metal body and a stabilized zirconia coating on the work engaging surface of said body, said stabilized zirconia covering the entire work engaging portion of the body and being fused thereto.
3. A furnace conveyor element and the like comprising a work supporting ferrous body and a stabilized zirconia coating covering the work engaging surface of said body and being fixed thereto.
4. A furnace conveyor element and the like comprising a work supporting ferrous body, a nickel chromium alloy film on the work engaging portion of said body and bonded thereto and an outer coating of stabilized zirconia fixed to the nickel chromium alloy film over the entire work engaging surface of the body.

5. A furnace conveyor roll and the like comprising a work supported metal body and a coating of zirconia stabilized with calcium oxide covering the work engaging portion of said body and fused thereto.

6. A furnace conveyor element and the like comprising a work supporting ferrous body and a zirconia coating stabilized with calcium oxide on the work engaging surface of said body, said stabilized zirconia covering the entire work engaging portion of the body and being fused thereto.

7. A furnace conveyor element and the like comprising a ferrous body, a nickel chromium alloy film on the work engaging portion of said body and bonded thereto and an outer coating of zirconia stabilized with calcium oxide fused to the nickel chromium alloy film over the entire work engaging surface of the body.

8. A furnace conveyor element and the like comprising a ferrous body, a nickel chromium alloy film consisting essentially of between about 60%-80% nickel and between 40%-20% chromium on the work engaging portion of said body and bonded thereto and an outer coating of stabilized zirconia fixed to the nickel chromium alloy film over the entire work engaging surface of the body.

#### References Cited in the file of this patent

#### UNITED STATES PATENTS

|           |                |       |               |
|-----------|----------------|-------|---------------|
| 1,578,254 | Bennett        | ----- | Mar. 30, 1926 |
| 1,861,489 | Brooke et al.  | ----- | June 7, 1932  |
| 2,151,048 | Rowe           | ----- | Mar. 21, 1939 |
| 2,624,097 | Kistler        | ----- | Jan. 6, 1953  |
| 2,695,248 | Ornitz et al.  | ----- | Nov. 23, 1954 |
| 2,848,349 | Rechter et al. | ----- | Aug. 19, 1958 |

#### OTHER REFERENCES

Pages 109 and 110 of Bulletin 186 by the Department of the Interior (Bureau of Mines) in 1921 titled, "Investigations of Zirconium With Especial Reference to the Metal and Oxide," published by the U.S. Government Printing Office, Washington, D.C.